

Jan. 4, 1938.

G. W. HEWITT

2,104,483

PRESERVATIVE AND CONTACT COAT FOR LIGHT SENSITIVE DEVICES

Filed March 5, 1936



Fig. 2.



Fig. 3.



Fig. 4.



WITNESSES:

G. J. Weller.  
R. W. Bailey.

INVENTOR  
George W. Hewitt.  
BY  
F. W. Syle.  
ATTORNEY

## UNITED STATES PATENT OFFICE

2,104,483

PRESERVATIVE AND CONTACT COAT FOR  
LIGHT-SENSITIVE DEVICES

George W. Hewitt, Wilkinsburg, Pa., assignor to  
Westinghouse Electric & Manufacturing Com-  
pany, East Pittsburgh, Pa., a corporation of  
Pennsylvania

Application March 5, 1936, Serial No. 67,278

6 Claims. (Cl. 136—89)

My invention relates to preservative coatings and especially to preservative coatings for light-sensitive devices.

It is an object of my invention to provide a preservative coating for light-sensitive devices that will not chip or lift away from the surface.

Other objects of my invention will become apparent upon reading the following description and drawing wherein:

10. Figure 1 is a cross-sectional view through a light-sensitive cell having my preferred form of preservative coating thereon;

Fig. 2 is an enlarged detail view of the central portion of Fig. 1;

15. Fig. 3 is a top view of a translucent organic sheet in a form especially adapted to be incorporated in the preservative coating; and

20. Fig. 4 is a perspective view of powdered siliceous material for incorporation in my preserva-  
tive coating.

25. In many respects, this invention is an improvement in the copending application of E. D. Wilson for preservative and contact coatings for light-sensitive devices Serial No. 67,277, filed March 5, 1936.

My invention has particular application to the copper oxide type of light-sensitive device, and Fig. 1 illustrates a preferred type of this device. The cell has a base of copper 10 having a layer of 30 cuprous oxide 11 integrally formed thereon. A translucent layer 12 of a noble metal, such as gold, silver, or platinum, is sputtered thereon with the barrier plane 13 therebetween composed of an ionized gas layer. The particular construction and method of manufacture of this 35 type of device is more specifically described in the copending applications of E. D. Wilson, namely, Serial No. 578,399, filed December 1, 1931; Serial No. 4,285, filed January 31, 1935; and Serial No. 20,362, filed May 8, 1935.

On the noble metal surface is formed a resinous coating 14, preferably of the natural resin type. The natural resins readily available for such use are rosin, colophony, abietic acid, ester gum, or 45 glycerized rosin. I also prefer to incorporate in this resin coating a plasticizer, preferably of the wax or glycerine type. Those readily available are beeswax, paraffin, Japan wax, normal butyl phthalate, ethylene glycol or other glycol. These 50 plasticizers can range from 2% to 25% of the natural resin coating, but 12½% of plasticizer works excellently.

At the edge of the disc is a mass 15 of pow-  
dered conductive material, such as silver, zinc, 55 carbon or a low melting alloy, as more specifically

described in the aforesaid copending application of E. D. Wilson Serial No. 67,277 for the purpose of making electrical contact with the noble metal layer 12. A metal ring 16 presses down on the broad surface of the conducting portion of this 5 preservative coating.

A difficulty with the above-described type of cell has been the effect of extreme temperatures upon the preservative coating of the cell. At very high temperatures, the preservative coating 10 will become sticky, and at low temperatures, the coating will tend to chip off away from the noble metal film. I increase the temperature range between the sticky stage at warm temperatures and the chipping-off stage at cold temperatures 15 by incorporating one or more materials into the resinous coating. One of these materials is a highly translucent material, such as powdered siliceous material 18. Readily available material of this class may be mica, glass or quartz pow- 20 dered into granules or flakes. This powdered material may be anywhere from 1% to 20% of the resinous coating. This material toughens the resinous coating and enables it to better withstand extremes of temperature. 25

Another substance that is also helpful in preventing cracks and chips is the incorporation of an organic film of material 17 into the resinous coating. This film may have a cellulose base, but I prefer to use a fibrous webbing or sheet 30 especially of the soft thin absorbent type. Wood pulp, cotton, glass wool or asbestos cotton are suitable. My preference is especially for the soft thin absorbent paper material used as cushion sheets for stencil backing. 35

In case paper is used, it will probably be necessary to avoid covering up very much of the contact area 15 of the preservative coating. Fig. 3 illustrates such a sheet 17 with tabs 19 for conveniently locating the edge of the disc, although 40 these tabs are not necessary. If cloth is used, the contact material can pass through the texture of the cloth.

In coating the copper oxide disc having its noble metal layer 12, the natural resin and its 45 plasticizer, if that is incorporated also, is mixed with the desired proportion of siliceous material 18 illustrated in Fig. 4. This mixed powder is uniformly distributed over the entire surface of the disc. By means of a special masking de- 50 vice, the granulated low-melting alloy is deposited in an annular area around the outer edge of the resinous layer. The cell is then placed on a hot plate. The resinous coating fuses, and the alloy melts down, sinking through the molten resin 55

to make contact with the noble metal. The fiber sheet 17 is now placed centrally on the fused resinous coating and becomes integral with it. The annular ring 16 can then be placed to make 5 a broad electrical contact to the low melting alloy. A closed circuit can then be made with the annular ring 16 as the outer negative terminal, and the copper as the positive terminal of the cell. Any desired electrical instrument, as the 10 meter 20, or relay, can be inserted in this circuit. The cell is self-generating in response to light striking the upper surface of the copper oxide surface and the electrons given off will pass the barrier plane 13 into the noble metal translucent 15 layer.

Although I have shown and described certain specific embodiments of my invention, I am fully aware that many modifications thereof are possible. My invention, therefore, is not to be restricted except insofar as is necessitated by the 20 prior art.

I claim as my invention:

1. In combination with a translucent metal film, a protective transparent coating therefor 25 comprising a resin from the group consisting of rosin, colophony, abietic acid, ester gum or glycerized rosin, a plasticizer from the group consisting of beeswax, paraffin, Japan wax, normal butyl, phthalate, ethylene glycol or other 30 glycol, and a translucent reinforcing material from the group consisting of mica, glass or quartz and a material from the group consisting of wood pulp, cotton, glass wool and asbestos cotton.

2. In combination with a translucent metal 35 film, a protective transparent coating therefor comprising a resin from the group consisting of rosin, colophony, abietic acid, ester gum or glycerized rosin, a plasticizer from the group consisting of beeswax, paraffin, Japan wax, normal butyl phthalate, ethylene glycol or other glycol, and a translucent reinforcing material from the 40 group consisting of mica, glass and quartz.

3. A photo-electric cell comprising copper having at least a portion of its surface oxidized, a 45 translucent coat of metal covering said oxidized

surface and a protective translucent coating therefor comprising a resin from the group consisting of rosin, colophony, abietic acid, ester gum or glycerized rosin, a plasticizer from the group consisting of beeswax, paraffin, Japan wax, normal butyl phthalate, ethylene glycol or other glycol, and a translucent reinforcing material from the group consisting of mica, glass or quartz and a material from the group consisting of wood pulp, cotton, glass wool and asbestos cotton. 5 10

4. A photo-electric cell comprising copper having at least a portion of its surface oxidized, a translucent coat of metal covering said oxidized surface and a protective translucent coating 15 therefor comprising a resin from the group consisting of rosin, colophony, abietic acid, ester gum or glycerized rosin, a plasticizer from the group consisting of beeswax, paraffin, Japan wax, normal butyl phthalate, ethylene glycol or other 20 glycol, and a translucent reinforcing material from the group consisting of mica, glass, quartz.

5. In combination with a translucent metal film, a protective transparent coating therefor 25 comprising a resin from the group consisting of rosin, colophony, abietic acid, ester gum or glycerized rosin, a plasticizer from the group consisting of beeswax, paraffin, Japan wax, normal butyl phthalate, ethylene glycol or other glycol, and a translucent reinforcing material from the 30 group consisting of wood pulp, cotton, glass wool and asbestos cotton.

6. A photo-electric cell comprising copper having at least a portion of its surface oxidized, a translucent coat of metal covering said oxidized 35 surface and a protective translucent coating therefor comprising a resin from the group consisting of rosin, colophony, abietic acid, ester gum or glycerized rosin, a plasticizer from the group consisting of beeswax, paraffin, Japan wax, normal butyl phthalate, ethylene glycol or other 40 glycol, and a translucent reinforcing material from the group consisting of wood pulp, cotton, glass wool and asbestos cotton.

GEORGE W. HEWITT. 45